

## UNITED STATES PATENT OFFICE

2,195,881

## REFRACTORY PANEL SHEET

Clements Batcheller, Glens Falls, N. Y., assignor  
to Allegheny Ludlum Steel Corporation, Pitts-  
burgh, Pa., a corporation of Pennsylvania

No Drawing. Application May 21, 1937,  
Serial No. 144,031

3 Claims. (Cl. 106—24)

My invention relates to refractory panels, and particularly to panels which, although they are hard and have comparatively high structural strength, are nevertheless of low specific gravity, whereby they are particularly adapted for use in connection with the interior construction of ships, railroad cars, aircraft, and the like, where low weight is absolutely necessary. Another object of my invention is to provide a product of this kind in which waste asbestos fibers of a grade heretofore considered unsuitable for use in standard types of cement-asbestos hard-pressed sheets may be employed and particularly to a panel board or sheet which can be produced on a cylinder press.

Many grades of asbestos fibers while entirely satisfactory in the matter of tensile strength, etc., cannot be used in the manufacture of sheet products of the character contemplated hereunder when formed upon a cylinder press by reason of the presence of talc which retards or even entirely prevents the successful removal of the felted plastic sheet from the cylinder drum of the machine, due to excessive sticking.

I have discovered that it is possible to produce my products to high degrees of strength from extremely low grade asbestos fibers and that the presence therein of talc in any reasonable quantity has no detrimental effect upon either the machine formation of the product or its ultimate strength and quality.

By forming my products largely from calcined diatomaceous earth, which weighs only from 10 to 16 pounds per cubic foot, not only is a very light product produced but one which is capable of withstanding extremely high temperatures without disintegrating. The diatomaceous earth may be either granular or finely ground, and a typical formula which I have found highly satisfactory is as follows:

|                                                                      | Parts   |
|----------------------------------------------------------------------|---------|
| Portland cement                                                      | 300     |
| Calcined diatomaceous earth                                          | 700     |
| Calcined magnesite                                                   | 200     |
| 45 Bentonite clay (200 mesh)                                         | 150     |
| Waste asbestos fibers (either with or without talc as an adulterant) | 250-300 |
| Water to produce a workable consistency                              |         |

The procedure followed in making my products from the above formula is substantially the well known Hatschek process which employs a wet cylinder press and is widely used in the formation of cement-asbestos products. Sheets or panels made from the above formula will with-

stand an applied temperature up to about 2000° F. without superficial crazing or spalling and, what is most important, without reducing the structural integrity of the product to a point where failure is indicated. Similar products made by any mechanical procedure when composed principally of Portland cement and mineral fibers become utterly useless at temperatures of the order of about 1500° F. The ordinary cement-asbestos products, for example, when subjected to 10 temperatures of the order of about 1000° F. and over break down rapidly. This is due in part to the calcination of the asbestos fibers and the release of chemical water which causes the products to explode under such conditions.

For some unexplained reason my products when formed from waste asbestos fibers containing appreciable quantities of talc are somewhat stronger and better than the same products formed from the highest grade of asbestos fibers such as those obtained from the areas of eastern Quebec, Canada although it is to be understood that my invention, of course, is not limited to the use of such waste fibers.

My products when formed to an appreciable thickness, say  $\frac{1}{2}$ " to 1" produce extremely efficient structural barriers against the passage of high heat.

The proportions of the ingredients given in the above formula may, of course, be varied to some degree, but the following limitations should be observed. The diatomaceous earth should be maintained substantially in excess of any other ingredient and the diatomaceous earth and bentonite combined should constitute 50% or 35 more, by weight, of the composition in order to provide a product of low specific gravity combined with resistance to high heat. Increasing the magnesite content and reducing the Portland cement content will enhance the structural strength of the product, and vice versa, while the bentonite content, due to the fact that it expands, when wet, to as much as fourteen times its original volume, preferably does not exceed about 10%, by weight, of the composition. However, the total cement content, that is the Portland cement and magnesite content combined, should be at least 25%, by weight, although more than 35% will probably not be desirable in any case.

What I claim is:

1. A refractory panel sheet characterized by its comparatively low specific gravity and its high resistance to crazing, spalling and structural disintegration under applied heat up to temperatures of the order of about 2000° F., said sheet

containing, by weight, the following ingredients, in about the proportions stated—

|                      | Parts   |
|----------------------|---------|
| Portland cement      | 300     |
| 5 Diatomaceous earth | 700     |
| Magnesium hydrate    | 200     |
| Bentonite            | 150     |
| Asbestos fibers      | 250-300 |

- 10 2. A refractory panel sheet characterized by its comparatively low specific gravity and its high resistance to crazing, spalling and structural disintegration under applied heat up to temperatures of the order of about 2000° F., and containing 15 diatomaceous earth, asbestos fibers, Portland cement, magnesium hydrate and bentonite; the weight of the diatomaceous earth content being substantially in excess of that of any other ingredient, and with the bentonite constituting

50% or more by weight of the sheet; the combined weight of the Portland cement and magnesium hydrate contents constituting from about 25% to 35% of the weight of the product, and the balance being principally asbestos fibers.

3. A refractory panel sheet characterized by its comparatively low specific gravity and its high resistance to crazing, spalling and structural disintegration under applied heat up to temperatures of the order of about 2000° F., and containing diatomaceous earth, asbestos fibers, Portland cement, magnesium hydrate and bentonite; the diatomaceous earth content constituting at least 40% of the total weight of the sheet, the Portland cement and magnesium hydrate contents 10 combined constituting at least 25% of said total weight, and the balance being substantially bentonite and asbestos fibers.

CLEMENTS BATCHELLER.